

R. A. HADFIELD AND A. G. MCK. JACK,  
MANUFACTURE OF ARMOR PIERCING PROJECTILES, SHELLS, AND OTHER HOLLOW BODIES,  
APPLICATION FILED MAY 24, 1920.

1,358,199.

Patented Nov. 9, 1920.

2 SHEETS—SHEET 1.

Fig. 1.



Fig. 6.



Fig. 7.



Inventors.

By Robert A. Hadfield,  
A. G. M. K. Jack.

J. Rose Millward  
Attorney.

R. A. HADFIELD AND A. G. MCK. JACK.  
MANUFACTURE OF ARMOR PIERCING PROJECTILES, SHELLS, AND OTHER HOLLOW BODIES.  
APPLICATION FILED MAY 24, 1920.

1,358,199.

Patented Nov. 9, 1920.

2 SHEETS—SHEET 2.

Fig. 2.



Fig. 4.



Fig. 3.



Fig. 5.



Inventors  
Robert A. Hadfield  
A. G. Mck. Jack.  
By

J. M. McLean  
Attorney

# UNITED STATES PATENT OFFICE.

ROBERT ABBOTT HADFIELD, OF WESTMINSTER, AND ALEXANDER GEORGE MCKENZIE JACK, OF BRINCLIFFE, SHEFFIELD, ENGLAND,

## MANUFACTURE OF ARMOR-PIERCING PROJECTILES, SHELLS, AND OTHER HOLLOW BODIES.

1,358,199.

Specification of Letters Patent.

Patented Nov. 9, 1920.

Application filed May 24, 1920. Serial No. 383,922.

To all whom it may concern:

Be it known that we, SIR ROBERT ABBOTT HADFIELD, Baronet, F. R. S., and ALEXANDER GEORGE MCKENZIE JACK, subjects of the 5 King of Great Britain and Ireland, residing, respectively, at the city of Westminster, England, and Brincliffe, Sheffield, in the county of York, England, have invented Improvements in or Relating to the Manufacture of Armor-Piercing Projectiles, Shells, and other Hollow Bodies, of which the following is a specification.

In the manufacture of armor piercing projectiles, shells, and other hollow bodies 15 by what is known as the extrusion process, that is to say, by piercing a central longitudinal hole in a solid metal blank by means of a longitudinally movable punch while the blank is held in a heated state within a stationary die or container, the wall of the projectile, shell or other hollow body is formed by metal displaced by the punch and caused to flow through an annular space left between the punch and the die or container.

20 In this extrusion process the metal constituting the wall of the armor piercing projectile, shell or other hollow body (hereinafter referred to as a shell) is caused to flow longitudinally in an outward direction and is not subjected to any compressive action that will cause lateral or radial movement of the metal except at the pointed free end portion of the punch where lateral outward displacement of the metal to form the 25 wall takes place. Consequently, the metal constituting the wall of the shell is not worked to the fullest extent, that is to say, the particles thereof are not subjected to such a degree of pressure and are not caused 30 to move relatively to one another to such an extent, as is necessary and desirable to enable the best physical characteristics, which it is possible to impart to the metal used, to be developed, particularly when the metal is 35 40 45 steel, for instance nickel chromium steel.

Now the present invention has for its object to enable the metal constituting the wall of a shell produced by the extrusion process to be worked to a greater extent than heretofore, and in a simple, quick, effective and economical manner, without drawing the shell through dies, so that the physical characteristics of the metal constituting such wall shall be considerably improved as com-

pared with those possessed by the metal of 55 the wall of the shell after the completion of the usual extrusion process.

For this purpose, in the manufacture of a shell according to the present invention, the wall thereof is subjected while supported externally but not internally and while at a suitable temperature, to endwise compression so as to cause the metal of which it is compressed to flow longitudinally backward toward the base of the shell and radially inward throughout the length of the wall or the greater portion thereof.

According to one mode of making a shell according to the invention, the wall of the shell is produced by the extrusion process in 70 the manner hereinbefore described but instead of making the wall of the shell of a thickness such that when the interior of the shell has been machined, the wall will be of the required finished thickness, that is to say, 75 instead of making the wall of the shell of a thickness of the completed forging at one pressing or extrusion, it is made by the extrusion process of less thickness than that required in the completed forging. Such an 80 extrusion process is herein called the modified extrusion process to distinguish it from the ordinary extrusion process referred to. The wall of the shell thus produced is afterward made of greater thickness by subjecting it, while supported externally but not internally and at a suitable temperature, to compression in a longitudinal direction so that the metal is caused to flow in the reverse 85 longitudinal direction to that in which it 90 flowed during the modified extrusion process and is simultaneously caused to flow in the inward radial direction, throughout the length of the wall or the greater portion thereof. In this way the metal comprising 95 the wall of the shell is worked in an effectual and advantageous manner for the purpose hereinbefore set forth.

In carrying out this mode of making a shell the shell is produced by piercing a 100 solid metal blank by the extrusion process but with a thinner wall than required in the completed forging and the extruded wall, while at a suitable temperature and while held within a die or container, is subjected 105 to endwise compression, as by forcing a plunger against its outer free end while it is unsupported internally, so that the metal

of the wall will be caused to flow both longitudinally backward and radially inward, the length of the wall being correspondingly reduced. By this means the metal will be 5 set up or caused to flow inwardly to substantially a similar extent throughout the whole length of the cavity in the shell, so that the cavity, after compression of the wall, will be of substantially the desired form, 10 that is to say, approximating to that of the required finished shape of the cavity with sufficient allowance for machining.

The invention can however advantageously be applied to the extruded wall of a 15 shell whatever may be its thickness in relation to that of the wall of the completed forging.

In the accompanying illustrative drawings, Figure 1 shows partly in side elevation 20 and partly in vertical section, and more or less diagrammatically, apparatus suitable for carrying the invention into practice.

Figs. 2, 3, 4 and 5 are similar views to Fig. 1 showing different stages in the process 25 of manufacturing a shell.

Figs. 6 and 7 are similar views to Fig. 5 showing modifications.

In carrying out the invention for the manufacture of say armor piercing projectiles 30 or high explosive shells, a solid cast steel blank *a*, (Fig. 1) heated to a suitable forging temperature, is placed in a die or container *b* and after being forced therein by a plunger *c* to cause it to properly fit the container *b* as usual, is pierced longitudinally 35 by a punch *d*, as shown in Fig. 2, operated hydraulically, so as to form a shell blank having an extruded wall *e* as heretofore. Instead however of using a punch *d* having a 40 diameter only appreciably smaller than that of the desired finished cavity in the shell, subsequently produced by machining, the punch *d* is made of a diameter substantially larger than that of the desired finished cavity 45 so as to form a thinner wall than is required in the completed forging. By this means, considerably more work is done upon the material than would otherwise be the case. After this modified extrusion process 50 is finished, the punch *d* is removed and the wall *e* of the shell, while still at a high temperature and held within the container *b* is, as shown in Fig. 3, subjected to the endwise pressure of a longitudinally movable 55 hydraulically operated plunger *f* whereby it is shortened, the metal composing it flowing longitudinally backward and radially inward, say from the position shown in dotted lines at *g* to the position shown approxi- 60 mately by the full lines *h*, thereby causing an additional advantageous working of the metal composing it and reducing the cavity or core *i* in the shell to a diameter and form approximating to that of the required 65 forged dimensions. The form of the cavity

or core *i* may, if desired, or when necessary, and as shown in Fig. 4 be rectified to the exact forged form required, by means of a rectifying punch or former *k* of the correct dimensions that is forced into it after the 70 compression stage above described is completed. Or, as shown in Fig. 5, the rectifying punch may be replaced by a punch or former *k*<sup>1</sup> that is of the required finished forged dimensions of the cavity in the shell 75 and is slidably supported within the hollow compression plunger *f*, so that when the plunger is lowered on to the wall of the extruded shell, the former *k*<sup>1</sup> will enter the cavity of the shell and be centrally supported 80 therein by the conical lower end thereof and the plunger will descend over it and compress the wall of the shell closely around it. Or, instead of making the plunger *f* and former *k*<sup>1</sup> separately, as in Fig. 5, they may, 85 as shown in Fig. 6, be made in one piece, or as shown in Fig. 7, in separate pieces rigidly fixed together, the former *k*<sup>1</sup> in this case coming to the bottom of the cavity and insuring the cavity being of the required finished forged dimensions when the plunger *f* has completed its downstroke. 90

The final form of the cavity or core *i* is, in each case, produced by machining the inner surface of the wall. 95

In this manner the wall of the shell is, in the first operation (Fig. 1) given considerably greater work than is usually the case, and in the second operation (Fig. 2) the further working effects an additional improvement in the physical properties of the material composing the wall of the shell. 100

The extrusion and compression or setting up processes described may be effected in quick succession without removal of the extruded shell from the container until the whole operation is finished. The extruded shell may however be removed from the container and reheated should this become necessary or desirable and afterward be replaced in the container or placed in another container and subjected to the compression or setting up process. 110

Although it is preferred to make the shell by extrusion with a wall of less thickness 115 than that required in the completed forging before subjecting it to compression, to cause movement of the metal in a longitudinal backward direction and in an inward direction as hereinbefore described, such compression could, as hereinbefore stated, advantageously be applied to the wall of an extruded shell made of any thickness, say of a thickness corresponding to that of the required finished forged dimensions of the 120 shell. In this case, the greater thickness of the wall produced by the endwise compression, may be reduced to the required thickness by another punching operation, or by 125 machining. 130

The plungers *c* and *f* and punch *d* may, as indicated in Fig. 1, be carried by a slide or cross-head *j* that is capable of being traversed horizontally in a guideway in the 5 lower side of the head *l* of the ram *m* of a vertically arranged hydraulic cylinder *n*. Or they may each be otherwise arranged.

What we claim is:—

1. In the manufacture of a shell, subjecting the wall of the shell while supported externally but not internally and while at a suitable temperature, to endwise compression so as to cause the metal of which it is composed to flow longitudinally backward toward the base of the shell and radially inward throughout the greater portion of the length of the wall, substantially as described for the purpose set forth.
2. In the manufacture of a shell by the extrusion process, forming the wall of the shell by the extrusion process of less thickness than that required in the completed forging and afterward subjecting such wall, while supported externally but not internally and 25 in a heated condition, to endwise compression toward the base of the shell so as to cause the metal of which it is composed to flow in the reverse longitudinal direction to that in which it flowed during the extrusion process and also to flow in an inward radial direction, substantially as described.
3. In the manufacture of a shell, subjecting the wall of the shell while supported externally but not internally and while at a suitable temperature to endwise compression so as to cause the metal of which it is composed to flow longitudinally backward toward the base of the shell and radially inward throughout the greater portion of the 35 length of the wall, and rectifying the form of the cavity of the shell to insure that it shall correspond to the exact forged form and dimensions required.
4. In the manufacture of a shell, subject-

ing the wall of the shell while supported externally but not internally and while at a suitable temperature, to endwise compression so as to cause the metal of which it is composed to flow longitudinally backward toward the base of the shell and radially inward throughout the greater portion of the length of the wall, and causing the inner surface of the resulting cavity of the shell to assume the exact forged form and dimensions required by finally arresting the radial 50 inward movement of the metal when such form and dimensions are attained.

5. In the manufacture of a shell, subjecting the wall of the shell while supported externally but not internally and while at a suitable temperature, to endwise compression so as to cause the metal of which it is composed to flow longitudinally backward toward the base of the shell and radially inward throughout the greater portion of the 55 length of the wall, the metal flowing radially inward being finally forced around and against a former, thereby insuring that the cavity of the shell is of the exact forged form and dimensions required.

6. In the manufacture of a shell, subjecting the wall of the shell while supported externally but not internally and while at a suitable temperature, to endwise compression so as to cause the metal of which it is 70 composed to flow longitudinally backward toward the base of the shell and radially inward throughout the greater portion of the length of the wall, and rectifying the form of the resulting cavity of the shell by radial 75 compression of the metal of the wall by the action of an internal support.

Signed at London in the county of London England this twenty ninth day of April 1920.

ROBERT ABBOTT HADFIELD.

ALEXANDER GEORGE MCKENZIE JACK.